

# United States Patent [19]

McComas et al.

[11] 4,235,943

[45] Nov. 25, 1980

[54] THERMAL SPRAY APPARATUS AND METHOD

[75] Inventors: Charles C. McComas, Stuart; Larry S. Sokol; Earl M. Hanna, both of West Palm Beach, all of Fla.

[73] Assignee: United Technologies Corporation, Hartford, Conn.

[21] Appl. No.: 13,944

[22] Filed: Feb. 22, 1979

## Related U.S. Application Data

[60] Continuation of Ser. No. 808,226, Jun. 20, 1977, abandoned, which is a continuation of Ser. No. 654,674, Feb. 2, 1976, abandoned, which is a division of Ser. No. 512,585, Oct. 7, 1974, abandoned.

[51] Int. Cl.<sup>2</sup> ..... B05D 1/00; B05D 1/08

[52] U.S. Cl. ..... 427/34; 427/191;  
427/192

[58] Field of Search ..... 427/34, 180, 191, 192

[56]

## References Cited

### U.S. PATENT DOCUMENTS

3,145,287 8/1964 Siebein et al. .... 219/75  
4,146,654 3/1979 Guyonnet ..... 427/423 X

Primary Examiner—Bernard D. Pianalto  
Attorney, Agent, or Firm—Robert C. Walker

[57]

## ABSTRACT

A thermal spray method capable of directing plasticized powders against a substrate for deposition of a protective coating thereon is disclosed. Various structural details of the apparatus described enable the attainment of high particle velocities without melting the particles. The method is built around the concept of reducing the temperature of a hot plasma stream after the hot plasma stream is generated. Coating particles are injected into the hot plasma stream only after the medium is cooled. In detailed embodiments, a generated plasma is cooled by the addition of a diluent gas or by passing the generated plasma through an elongated heat exchanger upstream of the point at which the powders are to be injected. The plasma is accelerated after the plasma is cooled to recover velocity lost in the cooling step.

9 Claims, 1 Drawing Figure





## THERMAL SPRAY APPARATUS AND METHOD

This is a continuation of application Ser. No. 808,226, filed June 20, 1977 which is a continuation of application Ser. No. 654,674, filed Feb. 2, 1976 which is a divisional application of Ser. No. 512,585, filed Oct. 7, 1974, now abandoned.

## BACKGROUND OF THE INVENTION

The present invention relates in general to the coating arts and more particularly, to the production of coatings by thermal spray techniques.

Plasma spraying devices and techniques are well known in the art for depositing protective coatings on underlying substrates. One known device is illustrated in U.S. Pat. No. 3,145,287 to Siebein et al entitled "Plasma Flame Generator and Spray Gun." In accordance with the teaching of the Siebein et al patent, a plasma-forming gas forms a sheath around an electric arc, constricts and extends the arc part way down the nozzle. The gas is converted to a plasma state and leaves the arc and nozzle as a hot free plasma stream. Powders are injected into the hot free plasma stream and propelled onto the surface of the substrate to be coated.

A prior art device, such as that illustrated by Siebein et al, is employed in the apparatus of the present invention to generate a hot plasma stream and is identified as item 6 of the Drawing.

U.S. Pat. Nos. 3,851,140 to Coucher entitled "Plasma Spray Gun and Method for Applying Coatings on a Substrate" and 3,914,573 to Muehlberger entitled "Coating Heat Softened Particles by Projection in a Plasma Stream of Mach 1 to Mach 3 Velocity" disclose contemporaneous coating technology. Both contemporaneous patents are common with Siebein et al in that coating powders are introduced immediately downstream of the point at which the plasma is generated. Physically, the point of injection in each case is at the downstream end of the anode within which the plasma is generated.

In addition to the Siebein et al and Muehlberger structures, Coucher employs a tubular nozzle downstream of the point of powder injection. According to the Coucher specification heat fusible material is thermally liquified as it contacts the hot plasma and is ejected with the hot plasma through the tubular nozzle.

Although the methods and devices disclosed likely have utility in the coating industry, scientists and engineers continue to search for yet improved coating methods and techniques.

## SUMMARY OF THE INVENTION

A primary aim of the present invention is to provide a method for depositing high quality coatings on a substrate. Thermal spray methods having enhanced ability to accelerate coating particles within a plasma stream is sought, and a collateral objective is to enable acceleration of such particles in a plasticized state.

According to the method of the present invention a hot plasma stream of a plasma generator is cooled to enable longer residence times of coating particles in the stream.

According to a more detailed method the plasma stream is accelerated after the plasma has been substantially cooled in order to recover stream velocity lost in the cooling process.

In the practice of at least one embodiment of the invention, a cooled nozzle extension assembly adapted to mate with conventional plasma spray equipment is fabricated with an aerodynamically efficient passageway through which the hot plasma may be passed and into which the coating powders may be introduced at a selected location or locations along the passageway. In operation thereof, helium is utilized as the plasma gas.

In the practice of another embodiment of the invention, a nozzle extension assembly adapted to mate with conventional plasma spray equipment includes means for injecting a diluent gas into the hot plasma in the passageway to cool the plasma stream prior to the location at which coating powders are injected.

A major advantage of the method of the present invention is an ability to generate optimum coating structures, in a variety of coating systems if desired, with excellent adherence and density. Increasing the residence time in the plasma increases the velocity of the coating powders carried. Recovering velocity lost in the cooling step increases the velocity differential between the plasma stream and the injected powders. These advantages are, moreover, achieved with concurrent improvements in process economy and safety.

The foregoing, and other objects, features and advantages of the present invention will become more apparent in the light of the following detailed description of the preferred embodiment thereof as shown in the accompanying drawing.

## BRIEF DESCRIPTION OF THE DRAWING

The drawing depicts plasma spray apparatus of the type capable of performing the teachings of this invention.

## DESCRIPTION OF THE PREFERRED EMBODIMENTS

The plasma spray apparatus shown in the drawing corresponds to that which has been actually used in the deposition of coatings according to the present invention.

A spray nozzle extension assembly 2 is adapted to fit around the nozzle 4 of a standard plasma spray gun 6 of the type having a cylindrical electrode to which an electric arc is struck in the formation of a hot plasma stream and through which the hot plasma stream is flowable and of the type including means for cooling the cylindrical electrode, such as the METCO 3MB Plasma Gun with GP Nozzle. The nozzle extension assembly comprises a tubular finned member 8 having a passageway 10 extending therethrough. As shown, the finned member is formed of a material of high thermal conductivity, such as copper and is surrounded by a steel water jacket 14 having a cooling water inlet 16 and outlet 18. The cooling fluid passing through the water chamber 19 cools the finned member preventing melting or other heat damage due to the hot plasma flowing through the passageway 10 during operation of the apparatus. In its traverse through the passageway in the cooled finned member, the hot plasma itself undergoes substantial cooling.

In this apparatus in the interest of maintaining a high gas velocity the passageway 10 has been shaped for aerodynamic efficiency, utilizing an inlet portion 20, a nozzle portion 22 and an outlet portion 24. Generated plasma is cooled in the inlet portion 20 and is accelerated in the nozzle portion 22. Coating powders to be sprayed are introduced downstream of the inlet portion

whereat the plasma has been cooled. The particular assembly shown is 6.3 inches in length with an inlet portion  $4 \times 0.215$  inches, a nozzle portion about 0.25 inch long having a throat diameter of 0.14 inch, and an outlet portion having a diameter of 0.15 inch. Thus, the nozzle is convergent/slightly divergent.

Typically, it is desirable to provide the powders to the surface to be coated, not only at high velocity and heated, but in a plastic rather than molten condition. As the plasma gas traverses the passageway it is cooled and, accordingly, introduction of the powders at a downstream location will generally result in a reduced heating of the powders because the temperature is lower than the upstream temperature. Accordingly, the nozzle is fabricated to provide sufficient length to substantially reduce the plasma temperature in the nozzle. Thus, as the word "elongated" is used herein, it will be understood to mean sufficient length to provide substantial cooling of the plasma. From the foregoing, it will be seen that in the present invention the coating powders are exposed in a relatively low temperature/long time cycle as contrasted with a high temperature/short time cycle in conventional plasma spray operations.

The nozzle extension assembly is provided with an access port or ports, 40 and 42 in the drawing, through which powder may be introduced into the plasma gas stream. The location of these powder access ports will depend upon the powders being sprayed and the particular process parameters and apparatus being utilized. Basically, however, the location is selected to provide the correct heating of the powders.

In the spraying of nickel/aluminum in the apparatus described, the powders are admitted in an inert carrier gas through access port 42 which is a 1/16 inch hole located about 3.5 inches downstream from the nozzle extension inlet or just upstream of the nozzle portion.

One or more access ports can be utilized for the introduction of differing powder compositions where such powders are to be sprayed concurrently or sequentially, or for the introduction of powders of the same composition where the processing parameters are to be changed. The formation of graded coatings by gradually phasing in one composition while phasing out another thereby eliminating a planar interface between the compositions is readily achieved.

As has been previously discussed, powder temperature can be readily controlled in a given system by careful selection of the axial location along the passageway where the powders are admitted to the hot gas stream. The apparatus is also readily adaptable to other means of powder temperature control. Access port 40 or some other port can, for example, be utilized for the admission of a temperature-modifying, or diluent gas to the plasma stream. This temperature-modifying gas may simply be a cold gas stream of the plasma gas composition or may be one which alters the heat transfer characteristics or some other property of the plasma.

As shown, the nozzle extension assembly comprises apparatus distinct from the plasma gun itself. This particular construction was selected for reasons of practicality to permit utilization of the present invention with existing plasma equipment. There is, of course, no reason why the extended nozzle cannot be integral with the gun itself. Also although the finned member 8 is shown formed as a single piece, various portions thereof may preferably be formed as separate members either to permit adaption of the assembly to alternative coating

operations or equipment, or simply to facilitate repairs or replacement of parts as they wear in use.

Usually to develop the optimum phase structure in the applied coating it is advantageous to have the powder particles impacting the surface to be coated in a plastic condition, but at as low a temperature as possible. However, the cooler the particles the higher the impact velocity must be to generate the maximum density and adherence. Thus, there is a considerable advantage to be gained through the provision of a capability of providing a high coating particle velocity.

Particle velocities are inherently limited by the gas velocity in the particular system being employed. In detonation spray processes, the particles are typically limited to shock wave velocities on the order of 2500 feet per second. Plasma spray guns, using argon as recommended by the manufacturers, may reach gas velocities up to 4000 feet per second. In the preferred embodiments of the present invention gas velocities of up to 12,000 feet per second or higher are possible.

Contrary to the usual industry practice, the use of helium as the plasma gas is preferred in the present invention. Although helium is known to have possible use in plasma spray operations, its light weight and poor heat transfer characteristics have resulted in industry discouraging its use in conventional plasma spray equipment. In the present invention its use is not only possible but advantageous.

In conventional equipment the gases exiting the plasma gun quickly disperse. Powders injected into such a stream reside therein for only a very short period of time. In these short residence times, the use of helium with its poor heat transfer capabilities, rather than argon, would increase the difficulty of imparting proper heat to the powders. This same short residence time and rapidly dispersing gas also aggravate the problem of providing the velocity component to the powders.

The preferred use of helium in the present invention provides controlled heating and a high velocity capability. In addition there are other advantages. With every coating process, it is essential to consider not only the effect of coating components and process parameters on the coating per se, but also their effect on the substrate being coated. Often the character of the substrate is such that certain temperatures of the substrate not be exceeded. The relatively poor heat transfer qualities of helium, as compared to argon for example, inherently result in a reduced heat transfer to the substrate.

In the conventional plasma spray operations, the dispersion of the heated gases results in a fairly large substrate area receiving heat, particularly areas where no coating is desired and which may be masked. In the present invention, there is a much greater degree of focus in the stream. Thus, smaller areas of the substrate are usually exposed at any one time to the hot gases and, hence, with a greater heat sink substrates remain cooler. As an additional benefit, it has been found that because of greater deposition area control the necessity and extent of masking is minimized; variations in coating structure and thickness are more controlled; and there is less powder waste, promoting economy.

Coating operations are also facilitated in another way through use of this invention. In use of a detonation gun operations are usually conducted with the operator positioned remote from the coating operation for safety reasons. With conventional plasma spray guns the exiting gas is at such a high temperature that eye damage from ultra-violet radiation can quickly occur and suit-

able eye protection is required. In the present invention, exit gas temperatures are reduced and the possibility of eye damage is lessened although, of course, suitable safety measures should be observed in any event.

In a conventional process, a part is typically prepared for coating by, first, masking to leave exposed only the areas to be coated; second, grit blasting; third, a cleanup to remove the effects of the grit blasting; and finally, a remasking. The present invention eliminates the need for many of these conventional steps in many cases. Since focusing is vastly improved the extent of masking is much reduced. Further, because particle velocities are very high, it has been found possible to eliminate the grit blasting operation and the masking and cleanup associated therewith. A simple surface wipe for degreasing with Freon has been found to be sufficient.

### EXAMPLE

| <u>Apparatus</u>          |                                                                                     |
|---------------------------|-------------------------------------------------------------------------------------|
| Plasma Gun Power Supply   | METCO 3MB with GP Nozzle PLASMADYNE<br>350 D.C. arc amps<br>50-56 D.C. arc volts    |
| Power Feeder              | S.S. AIRABRASIVE unit<br>(miniature grit blaster)<br>powder feed rate .357 lbs./hr. |
| Nozzle Extension Assembly | per drawing                                                                         |
| Powder (METCO 450)        |                                                                                     |
| Composition (wt. %)       | 95 percent nickel<br>5 percent aluminum<br>170 + 325 mesh (ASTM B214)               |
| Particle size             | helium                                                                              |
| Process Parameters        | 275 ft. <sup>3</sup> /min.                                                          |
| Plasma Gas                | 2-3 inches                                                                          |
| Gas Rate                  |                                                                                     |
| Gun to Substrate Distance |                                                                                     |
| Size of Focus             | 8 inch                                                                              |
| Substrate                 | titanium alloy                                                                      |
| Coating area              | flat washer                                                                         |

### Deposition

Using the hand held coating gun with attached nozzle extension assembly, a coating 0.008-0.010 inch in thickness was applied for galling and fretting resistance to one surface of the flat washer.

### Results

A coating density of well over 99 percent of theoretical density was achieved. This is in excess of that attainable in any conventional plasma process. Adherence was excellent. Repeated thermal shocking from high temperature resulted in no evidence whatsoever of cracking or flaking.

Although this invention has been described in detail with reference to certain examples and preferred embodiments for the sake of illustration, the invention in its broader aspects is not limited to such specific details but departures may be made from such details without departing from the principles of the invention and without sacrificing its chief advantages.

### What is claimed is:

1. A plasma powder spray method which comprises: generating a plasma; passing the plasma at high velocity through an elongated nozzle; cooling the plasma, forming a cooled plasma gas stream; accelerating the cooled plasma;

admitting coating powder to the cooled gas stream in the nozzle, providing sufficient powder residence time in the cooled gas stream to plasticize the powder and impart a high velocity thereto; and directing the plasticized powder to a surface to be coated and effecting a coating buildup thereon to the desired thickness.

2. A method according to claim 1 wherein: the plasma is a helium plasma.
3. A plasma powder spray method which comprises: generating a helium plasma at high temperature; passing the plasma at high velocity through an elongated nozzle; cooling the nozzle and the plasma passing therethrough forming a cooled plasma gas stream; accelerating the cooled plasma; admitting coating powder to be cooled gas stream in the nozzle, plasticizing the powder and imparting a high velocity thereto; and directing the plasticized powder to a surface to be coated and effecting a coating buildup thereon to the desired thickness.
4. A plasma powder spray method which comprises: forming a high temperature plasma gas in a plasma generator; discharging the high temperature plasma gas from the plasma generator at a high velocity; flowing the high temperature, high velocity plasma gas to an elongated nozzle downstream of the plasma generator; passing the high velocity plasma gas through the elongated nozzle; cooling the plasma in the elongated nozzle to form a cooled, high velocity plasma gas stream; accelerating the cooled plasma in the elongated nozzle; admitting coating powder to the cooled, high velocity gas stream in the nozzle, and providing sufficient powder residence time in the cooled, high velocity gas stream to plasticize the powder and impart a high velocity thereto; and directing the plasticized powder to a surface to be cooled and effecting a coating buildup thereon to the desired thickness.
5. A method according to claim 4 wherein: the plasma is a helium plasma.
6. A plasma powder spray method which comprises: generating a helium plasma at high temperature in a plasma generator; discharging the high temperature helium plasma from the plasma generator at a high velocity; passing the plasma at high velocity through an elongated nozzle; cooling the nozzle and the plasma passing therethrough forming a cooled plasma gas stream; accelerating the cooled plasma in the elongated nozzle; admitting coating powder to the cooled gas stream in the nozzle, plasticizing the powder and imparting a high velocity thereto; and directing the plasticized powder to a surface to be coated and effecting a coating buildup thereon to the desired thickness.
7. In a plasma spray method of the type in which coating powders to be deposited are carried in a plasma stream, the improvement which comprises: substantially cooling the plasma stream;

accelerating the plasma stream after the plasma stream has been cooled; and introducing coating powders into the plasma stream after the plasma stream has been cooled.

8. The invention according to claim 7 wherein the step of substantially cooling the plasma stream includes the steps of passing the plasma stream through the pas-

sageway of a tubular finned member and circulating a cooling fluid about the tubular finned member.

9. The invention according to claim 7 wherein the step of substantially cooling the plasma stream includes the step of introducing a diluent gas into the stream prior to the introduction of coating powders.

\* \* \* \* \*

10

15

20

25

30

35

40

45

50

55

60

65

UNITED STATES PATENT AND TRADEMARK OFFICE  
CERTIFICATE OF CORRECTION

PATENT NO. : 4,235,943

DATED : November 25, 1980

INVENTOR(S) : Charles C. McComas, Larry S. Sokol, Earl M. Hanna

It is certified that error appears in the above-identified patent and that said Letters Patent are hereby corrected as shown below:

Column 5, line 24 "Power" should be "Powder"

Column 6, claim 3, line 17 "be" should be "the"

**Signed and Sealed this**

*Seventh Day of April 1981*

[SEAL]

*Attest:*

RENE D. TEGTMEYER

*Attesting Officer*

*Acting Commissioner of Patents and Trademarks*